# EUROPEAN PATENT SPECIFICATION

(11) **EP 0 257 577 B1**
(45) Date of publication and mention of the grant of the patent: **23.10.1991**
(21) Application number: 87112145.5
(22) Date of filing: 21.08.1987
(51) Int. Cl.: B41M 5/26

(54) **N-alkyl- or n-aryl-aminopyrazolone merocyanine dye-donor element used in thermal dye transfer**
N-Alkyl- oder N-Arylaminopyrazolon-merocyanin-Farbstoff-Donor-Element für die thermische Farbstoffübertragung
N-alkyl- ou N-arylaminopyrazolone merocyanine, élément donneur de colorant utilisé pour le transfert thermique

(30) Priority: 22.08.1986 US 899273; 06.10.1986 US 915451; 08.06.1987 US 59443
(43) Date of publication of application: 02.03.1988
(73) Proprietor: EASTMAN KODAK COMPANY (a New Jersey corporation), Rochester, New York 14650 (US)
(72) Inventor: Byers, Gary Wayne, Rochester New York 14650 (US); Evans, Steven, Rochester New York 14650 (US); Weber, Helmut, Rochester New York 14650 (US)
(74) Representative: Brandes, Jürgen, Dr. rer. nat.

(56) References cited:
- EP-A- 0 257 578
- FR-A- 2 272 217
- PATENT ABSTRACTS OF JAPAN, vol. 10, no. 70 (M-462)[2127], 19 mars 1986, page 158 M 462; & JP-A-60 214 994 (RICOH K.K.) 28-10-1985

## Description

This invention relates to N-alkyl- or N-aryl-aminopyrazolone merocyanine dye-donor elements used in thermal dye transfer which have good stability to light.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to the cyan, magenta and yellow signals. The process is then repeated for the other two colors. A color hard copy is thus obtained which corresponds to the original picture viewed on a screen. Further details of this process and an apparatus for carrying it out are contained in U.S. Patent No. 4,621,271 by Brownstein entitled "Apparatus and Method For Controlling A Thermal Printer Apparatus," issued November 4, 1986.

One of the major problems in selecting a dye for thermal dye-transfer printing is to obtain good transfer efficiency to produce high maximum density. Another problem is to obtain such dyes which have good stability to light. Many of the dyes proposed for use are not suitable because they either yield inadequate transfer densities at reasonable coating coverages or have poor light stability.

It is an object of this invention to provide dyes which have high transfer densities used in thermal dye-transfer printing and which have good stability to light.

Japanese Patent Publication 60/214994 relates to cyanine or merocyanine dyes which are used in an image recording material. Those dyes, however, are not used in a thermal dye transfer system. Instead, those dyes are light bleachable, such as by flash exposure, to bleach or destroy the dye. Thus, those dyes undergo substantial photolysis or decomposition, when exposed to radiant energy. In addition, those dyes absorb at wavelengths substantially beyond the visible spectrum, unlike the dyes of the present invention.

These and other objects are achieved in accordance with the invention which comprises a dye-donor element comprising a support having thereon a dye layer characterized in that the dye comprises a 3-(N-alkyl- or N-aryl-amino)-2-pyrazolin-5-one merocyanine dye dispersed in a polymeric binder, the merocyanine dye being capable of transfer by diffusion to a dye-receiving element upon the application of heat and being incapable of substantial photolysis, the merocyanine dye being substituted or unsubstituted on the bridging methine carbon atoms. By saying that the dyes of the invention are "incapable of substantial photolysis" is meant that the dyes of the invention do not undergo any substantial decomposition when exposed to radiant energy.

By appropriate selection of substituents, the merocyanine dyes employed in the invention may be of magenta or yellow hue.

In a preferred embodiment of the invention, the merocyanine dye has the formula:
wherein:
R represents a substituted or unsubstituted alkyl group of from 1 to 6 carbon atoms such as methyl, ethyl, propyl, isopropyl, butyl, pentyl, hexyl or such alkyl groups substituted with hydroxy, acyloxy, alkoxy, aryl, cyano, acylamido, halogen, etc.; or a substituted or unsubstituted aryl group of from 6 to 10 carbon atoms such as phenyl, p-tolyl, m-chlorophenyl, p-methoxyphenyl, m-bromophenyl, o-tolyl, etc.;
R¹ and R² each independently represent hydrogen, with the proviso that only one of R¹ and R² may be hydrogen at the same time; a substituted or unsubstituted alkyl group of from 1 to 6 carbon atoms or a substituted or unsubstituted aryl group of from 6 to 10 carbon atoms, such as those discussed above for R; or R¹ and R² may be combined together with the nitrogen to which they are attached to form a heterocyclic ring system;
R³ is R;
n represents 0 or 1; and
Z represents the atoms necessary to complete a 5- or 6-membered substituted or unsubstituted heterocyclic ring such as 3H-indole, benzoxazole, thiazoline, benzimidazole, oxazole, thiazole, etc., and may include linking groups such as -CR₂-, -CR=CR-, -O-, -S-, -Te-, -Se-, or -NR-.

In a preferred embodiment of the invention, Z represents the atoms necessary to complete an indoline ring. In another preferred embodiment of the invention, R¹ and R² are both methyl. In another preferred embodiment of the invention, R³ is phenyl.

These dyes may be prepared by synthetic procedures similar to those described in copending Application Serial No. , by Byers and Chapman entitled "Merocyanine Dye-Donor Element Used in Thermal Dye Transfer", filed of even date herewith.

Compounds included within the scope of the invention include the following:

A dye-barrier layer comprising a hydrophilic polymer may be employed in the dye-donor element of the invention between its support and the dye layer to improve the density of the transferred dye.

The dye in the dye-donor element of the invention is dispersed in a polymeric binder such as a cellulose derivative, e.g., cellulose acetate hydrogen phthalate, cellulose acetate, cellulose acetate propionate, cellulose acetate butyrate, cellulose triacetate; a polycarbonate; poly(styrene-co-acrylonitrile), a poly(sulfone) or a poly(phenylene oxide). The binder may be used at a coverage of from 0.1 to 5 g/m².

The dye layer of the dye-donor element may be coated on the support or printed thereon by a printing technique such as a gravure process.

Any material can be used as the support for the dye-donor element of the invention provided it is dimensionally stable and can withstand the heat of the thermal printing heads. Such materials include polyesters such as poly(ethylene terephthalate); polyamides; polycarbonates; glassine paper; condenser paper; cellulose esters; fluorine polymers; polyethers; polyacetals; polyolefins; and polyimides. The support generally has a thickness of from 2 to 30 µm. It may also be coated with a subbing layer, if desired.

The reverse side of the dye-donor element may be coated with a slipping layer to prevent the printing head from sticking to the dye-donor element. Such a slipping layer would comprise a lubricating material such as a surface active agent, a liquid lubricant, a solid lubricant or mixtures thereof, with or without a polymeric binder.

The dye-receiving element that is used with the dye-donor element of the invention usually comprises a support having thereon a dye image-receiving layer. The support may be a transparent film such as a poly(ether sulfone), a polyimide, a cellulose ester such as cellulose acetate, a poly(vinyl alcohol-co-acetal) or a poly(ethylene terephthalate). The support for the dye-receiving element may also be reflective such as baryta-coated paper, polyethylene-coated paper, white polyester (polyester with white pigment incorporated therein), an ivory paper, a condenser paper or a synthetic paper such as duPont Tyvek®. In a preferred embodiment, polyester with a white pigment incorporated therein is employed.

The dye image-receiving layer may comprise, for example, a polycarbonate, a polyurethane, a polyester, polyvinyl chloride, poly(styrene-co-acrylonitrile), poly(caprolactone) or mixtures thereof. The dye image-receiving layer may be present in any amount which is effective for the intended purpose. In general, good results have been obtained at a concentration of from 1 to 5 g/m².

As noted above, the dye-donor elements of the invention are used to form a dye transfer image. Such a process comprises imagewise-heating a dye-donor element as described above and transferring a dye image to a dye-receiving element to form the dye transfer image.

The dye-donor element of the invention may be used in sheet form or in a continuous roll or ribbon. If a continuous roll or ribbon is employed, it may have only the dye thereon as described above or may have alternating areas of other different dyes, such as sublimable cyan, yellow, magenta and/or black or other dyes. Such dyes are disclosed in U.S. Patent 4,541,830. Thus, one-, two-, three- or four-color elements (or higher numbers also) are included within the scope of the invention.

In a preferred embodiment of the invention, the dye-donor element comprises a poly(ethylene terephthalate) support coated with sequential repeating areas of cyan, magenta and yellow dye, at least one of the dyes being a merocyanine dye as described above, and the above process steps are sequentially performed for each color to obtain a three-color dye transfer image. Of course, when the process is only performed for a single color, then a monochrome dye transfer image is obtained.

A thermal dye transfer assemblage of the invention comprises
a) a dye-donor element as described above, and
b) a dye-receiving element as described above,
the dye-receiving element being in a superposed relationship with the dye-donor element so that the dye layer of the donor element is in contact with the dye image-receiving layer of the receiving element.

The above assemblage comprising these two elements may be preassembled as an integral unit when a monochrome image is to be obtained. This may be done by temporarily adhering the two elements together at their margins. After transfer, the dye-receiving element is then peeled apart to reveal the dye transfer image.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought in register with the dye-receiving element and the process repeated. The third color is obtained in the same manner.

The following examples are provided to illustrate the invention.

### Example 1 - Yellow Dyes

A yellow dye-donor element was prepared by coating the following layers in the order recited on a 6 µm poly(ethylene terephthalate) support:
1) Dye-barrier layer of poly(acrylic) acid (0.16 g/m²) coated from water, and
2) Dye layer containing a yellow dye as identified in the following Table 1 (0.63 mmoles/m²), a cellulose acetate binder (40% acetyl) at a weight equal to 1.2X that of the dye, and FC-431® 3M Corp. (2.2 mg/m²), coated from a 2-butanone-cyclohexanone solvent mixture.
On the back side of the element was coated a typical slipping layer.

A dye-receiving element was prepared by coating a solution of Makrolon 5705® (Bayer AG Corporation) polycarbonate resin (2.9 g/m² in a methylene chloride and trichloroethylene solvent mixture on an ICI Melinex 990® white polyester support.

The dye side of the dye-donor element strip 0.75 inches (19 mm) wide was placed in contact with the dye image-receiving layer of the dye-receiver element of the same width. The assemblage was fastened in the jaws of a stepper motor driven pulling device. The assemblage was laid on top of a 0.55 inch (14 mm) diameter rubber roller and a TDK Thermal Head (No. L-133) and was pressed with a spring at a force of 8.0 pounds (3.6 kg) against the dye-donor element side of the assemblage pushing it against the rubber roller.

The imaging electronics were activated causing the pulling device to draw the assemblage between the printing head and roller at 0.123 inches/sec (3.1 mm/sec). Coincidentally, the resistive elements in the thermal print head were pulse-heated at increments from 0 to 8.3 msec to generate a graduated density test pattern. The voltage supplied to the print head was approximately 22v representing approximately 1.5 watts/dot (12 mjoules/dot) for maximum power.

The dye-receiving element was separated from the dye-donor element and the status A blue reflection density at the maximum density was read. The image was then subjected to "HID fading", 7 days, 50 Klux, 5400° K, 32°C, approximately 25% RH.
The percent density loss was then calculated. The following results were obtained:

The above results indicate that the merocyanine yellow dyes of the invention had better light stability than the control dyes.

### Example 2 - Yellow Dyes

Example 1 was repeated except that the following compounds listed in Table 2 were evaluated which do not have indoline moieties. They were compared to similar control dyes which do not have amino groups. The following results were obtained:

The above results again indicate that the merocyanine yellow dyes of the invention had better light stability than similar control dyes which did not have amino groups.

### Example 3 - Yellow Dyes

Example 1 was repeated except that the following compounds listed in Table 3 were evaluated. Four control yellow dyes were prepared and tested which are similar to dyes employed in the invention except that they have a 3-methyl instead of a 3-(N,N-dialkylamino) substitution on the 2-pyrazolin-5-one ring. The following results were obtained:

The above results indicate that the dyes employed according to the invention had higher transfer densities and much better light stability than similar control dyes which did not have amino groups.

### Example 4 - Magenta Dyes

Example 1 was repeated except that the following magenta compounds listed in Table 4 were evaluated and the Green Status A maximum density was measured. Three control magenta dyes were prepared and tested which are similar to dyes employed in the invention except that they have a 3-methyl instead of a 3-(N,N-dialkylamino) substitution on the 2-pyrazolin-5-one ring. The following results were obtained:

The above results indicate that the dyes employed according to the invention had much better light stability than similar control dyes which did not have amino groups.

## Claims

1. A dye-donor element for thermal dye transfer comprising a support having thereon a dye layer characterized in that the dye comprises a 3-(N-alkyl- or N-aryl-amino)-2-pyrazolin-5-one merocyanine dye dispersed in a polymeric binder, said merocyanine dye being capable of transfer by diffusion to a dye-receiving element upon the application of heat and being incapable of substantial photolysis, said merocyanine dye being substituted or unsubstituted on the bridging methine carbon atoms.

2. The element of Claim 1 characterized in that said 3-(N-alkyl- or N-aryl-amino)-2-pyrazolin-5-one merocyanine dye has the formula: wherein:
R represents a substituted or unsubstituted alkyl group of from 1 to 6 carbon atoms or a substituted or unsubstituted aryl group of from 6 to 10 carbon atoms;
R¹ and R² each independently represents hydrogen, with the proviso that only one of R¹ and R² may be hydrogen at the same time; a substituted or unsubstituted alkyl group of from 1 to 6 carbon atoms or a substituted or unsubstituted aryl group of from 6 to 10 carbon atoms; or R¹ and R² may be combined together with the nitrogen to which they are attached to form a heterocyclic ring system;
R³ is R;
n represents 0 or 1; and
Z represents the atoms necessary to complete a 5- or 6-membered substituted or unsubstituted heterocyclic ring.

3. The element of Claim 2 characterized in that Z represents the atoms necessary to complete an indoline ring.

4. The element of Claim 2 characterized in that R¹ and R² are both methyl.

5. The element of Claim 2 characterized in that R³ is phenyl.

6. The element of Claim 1 characterized in that said support comprises poly(ethylene terephthalate), the side of the support opposite the side having thereon said dye layer is coated with a slipping layer comprising a lubricating material, and said dye layer comprises sequential repeating areas of cyan, magenta and said yellow dye.

7. A thermal dye transfer assemblage comprising:
a) a dye-donor element comprising a support having thereon a dye layer comprising a dye dispersed in a polymeric binder, and
b) a dye-receiving element comprising a support having thereon a dye image-receiving layer,
said dye-receiving element being in a superposed relationship with said dye-donor element so that said dye layer is in contact with said dye image-receiving layer,
characterized in that said dye comprises a 3-(N-alkyl- or N-aryl-amino)-2-pyrazolin-5-one merocyanine dye, said merocyanine dye being capable of transfer by diffusion to a dye-receiving element upon the application of heat and being incapable of substantial photolysis, said merocyanine dye being substituted or unsubstituted on the bridging methine carbon atoms.

8. The assemblage of Claim 7 characterized in that said 3-(N-alkyl- or N-aryl-amino)-2-pyrazolin-5-one merocyanine dye has the formula: wherein:
R represents a substituted or unsubstituted alkyl group of from 1 to 6 carbon atoms or a substituted or unsubstituted aryl group of from 6 to 10 carbon atoms;
R¹ and R² each independently represents hydrogen, with the proviso that only one of R¹ and R² may be hydrogen at the same time; a substituted or unsubstituted alkyl group of from 1 to 6 carbon atoms or a substituted or unsubstituted aryl group of from 6 to 10 carbon atoms; or R¹ and R² may be combined together with the nitrogen to which they are attached to form a heterocyclic ring system;
R³ is R;
n represents 0 or 1; and
Z represents the atoms necessary to complete a 5- or 6-membered substituted or unsubstituted heterocyclic ring.

9. The assemblage of Claim 8 characterized in that Z represents the atoms necessary to complete an indoline ring.

10. The assemblage of Claim 8 characterized in that R¹ and R² are both methyl and R³ is phenyl.

## Revendications

1. Elément donneur de colorant utilisé dans le transfert thermique de colorant comprenant un support portant une couche de colorant caractérisé en ce que le colorant est un colorant mérocyanine 3-(N-alkyl-ou N-aryl-amino)-2-pyrazolin-5-one dispersé dans un liant polymère transférable par diffusion sur l'élément récepteur de colorant pendant le chauffage et peu sensible à la photolyse, colorant mérocyanine ayant une chaine de liaison méthinique substituée ou non.

2. Elément selon la revendication 1, caractérisé en ce que le colorant mérocyanine 3-(N-alkyl- ou N-aryl-amino)-2-pyrazolin-5-one correspond à la formule : où
R représente un groupe alkyle substitué ou non de 1 à 6 atomes de carbone ou un groupe aryle substitué ou non de 6 à 10 atomes de carbone ;
R¹ et R², chacun séparément, représente un atome d'hydrogène avec la condition suplémentaire que R¹ et R² ne peuvent pas représenter un atome d'hydrogène en même temps ; un groupe alkyle substitué ou non de 1 à 6 atomes de carbone ou un groupe aryle substitué ou non de 6 à 10 atomes de carbone ; ou R¹ et R² peuvent être combinés ensemble avec un atome d'azote pour former un système hétérocyclique ;
R³ est R ;
n représente 0 ou 1 ; et
Z représente les atomes nécessaires pour former un hétérocycle à 5 ou 6 membres substitué ou non.

3. Elément selon la revendication 2 caractérisé en ce que Z représente les atomes nécessaires pour former un cycle indoline.

4. Elément selon la revendication 2 caractérisé en ce que R¹ et R² sont tous les deux des groupes méthyle.

5. Elément selon la revendication 2 caractérisé en ce que R³ est un groupe phényle.

6. Elément selon la revendication 1 caractérisé en ce que le support est constitué de polytéréphtalate d'éthylène, le coté du support opposé au coté portant la couche de colorant est recouvert d'une couche favorisant le glissement comprenant un composé lubrifiant et, la couche de colorant comprend des zones séquencées de colorants cyan, magenta et jaune.

7. Assemblage pour le transfert thermique de colorant comprenant
a) un élément donneur de colorant comprennent un support portant une couche de colorant obtenue en dispersant le colorant dans un liant polymère, et
b) un élément récepteur de colorant comprenant un support portant une couche réceptrice d'image de colorant, cet élément récepteur de colorant étant superposé à l'élément donneur de colorant de manière que la couche de colorant soit en contact avec la couche réceptrice d'image de colorant, caractérisé en ce que le colorant est un colorant mérocyanine 3-(N-alkyl- ou N-aryl-amino)-2-pyrazolin-5-one dispersé dans un liant polymère transférable par diffusion sur l'élément récepteur de colorant pendant le chauffage et peu sensible à la photolyse, colorant mérocyanine ayant une chaine de liaison méthinique substituée ou non.

8. Assemblage selon la revendication 7 caractérisé en ce que le colorant mérocyanine 3-(N-alkyl- ou N-aryl-amino)-2-pyrazolin-5-one correspond à la formule : où
R représente un groupe alkyle substitué ou non de 1 à 6 atomes de carbon ou un groupe aryle substitué ou non de 6 à 10 atomes de carbone ;
R¹ et R², chacun séparément, représente un atome d'hydrogène avec la condition suplémentaire que R¹ et R² ne peuvent pas représenter un atome d'hydrogène en même temps ; un groupe alkyle substitué ou non de 1 à 6 atomes de carbone ou un groupe aryle substitué ou non de 6 à 10 atomes de carbone ; ou R¹ et R² peuvent être combinés ensemble avec un atome d'azote pour former un système hétérocyclique ;
R³ est R ;
n représente 0 ou 1 ;
Z représente les atomes nécessaires pour former un hétérocycle à 5 ou 6 membres substitué ou non.

9. Assemblage selon la revendication 8 caractérisé en ce que Z représente les atomes nécessaires pour former un cycle indoline.

10. Assemblage selon la revendication 8 caractérisé en ce que R¹ et R² sont tous les deux des groupes méthyle.

## Patentansprüche

1. Farb-Donorelement für die thermische Farbstoffübertragung mit einem Träger, auf den eine Farbstoffschicht aufgetragen ist, dadurch gekennzeichnet, daß der Farbstoff einen 3-(N-Alkyl- oder N-Aryl-amino)-2-pyrazolin-5-on-Merocyanin-farbstoff umfaßt, der in einem polymeren Binder dispergiert ist, der bei Einwirkung von Wärme durch Diffusion auf ein Farbstoff-Empfangselement übertragbar ist und praktisch keiner Photolyse unterliegt, und der an den eine Brücke bildenden Methin-Kohlenstoffatomen substituiert oder unsubstituiert ist.

2. Element nach Anspruch 1, dadurch gekennzeichnet, daß der 3-(N-Alkyl- oder N-Aryl-amino)-2-pyrazolin-5-on-Merocyanin-Farbstoff der folgenden Formel entspricht: in der bedeuten:
R eine substituierte oder unsubstituierte Alkylgruppe mit 1 bis 6 Kohlenstoffatomen oder eine substituierte oder unsubstituierte Arylgruppe mit 6 bis 10 Kohlenstoffatomen;
R¹ und R² jeweils unabhängig voneinander Wasserstoff, wobei gilt, daß R¹ und R² nicht gleichzeitig Wasserstoff sein können; eine substituierte oder unsubstituierte Alkylgruppe mit 1 bis 6 Kohlenstoffatomen oder eine substituierte oder unsubstituierte Arylgruppe mit 6 bis 10 Kohlenstoffatomen; oder R¹ und R² gemeinsam mit dem Stickstoffatom, an das sie gebunden sind, ein heterocyclisches Ringsystem;
R³ gleich R;
n gleich 0 oder 1 und
Z die Atome, die zur Vervollständigung eines 5- oder 6-gliedrigen substituierten oder unsubstituierten heterocyclischen Ringes erforderlich sind.

3. Element nach Anspruch 2, dadurch gekennzeichnet, daß Z für die Atome steht, die zur Vervollständigung eines Indolringes erforderlich sind.

4. Element nach Anspruch 2, dadurch gekennzeichnet, daß R¹ und R² jeweils Methylgruppen sind.

5. Element nach Anspruch 2, dadurch gekennzeichnet, daß R³ für eine Phenylgruppe steht.

6. Element nach Anspruch 1, dadurch gekennzeichnet, daß der Träger Poly(ethylenterephthalat) umfaßt, daß die Seite des Trägers, die der Seite mit der Farbstoffschicht gegenüberliegt, mit einer Gleitschicht beschichtet ist, die ein Gleitmittel enthält und daß die Farbschicht regelmäßig angeordnete, sich wiederholende Bezirke aus blaugrünem, purpurrotem und gelbem Farbstoff aufweist.

7. Zusammensetzung für die thermische Farbstoffübertragung mit
a) einem Farb-Donorelement mit einem Träger, auf dem sich eine Schicht befindet, die einen in einem polymeren Binder dispergierten Farbstoff enthält und
b) einem Farbstoff-Empfangselement mit einem Träger, auf dem sich eine Farbbild-Empfangsschicht befindet,
wobei Farbstoff-Empfangselement und Farb-Donorelement übereinander angeordnet sind, derart, daß sich die Farbstoffschicht in Kontakt mit der Farbbild-Empfangsschicht befindet, dadurch gekennzeichnet, daß der Farbstoff einen 3-(N-Alkyl- oder N-Aryl-amino)-2-pyrazolin-5-on-Merocyanin-farbstoff umfaßt, der in einem polymeren Binder dispergiert ist, der bei Einwirkung von Wärme durch Diffusion auf ein Farbstoff-Empfangselement übertragbar ist und praktisch keiner Photolyse unterliegt, und der an den eine Brücke bildenden Methin-Kohlenstoffatomen substituiert oder unsubstituiert ist.

8. Zusammensetzung nach Anspruch 7, dadurch gekennzeichnet, daß der 3-(N-Alkyl- oder N-Aryl-amino)-2-pyrazolin-5-on-Merocyanin-Farbstoff der folgenden Formel entspricht: in der bedeuten:
R eine substituierte oder unsubstituierte Alkylgruppe mit 1 bis 6 Kohlenstoffatomen oder eine substituierte oder unsubstituierte Arylgruppe mit 6 bis 10 Kohlenstoffatomen;
R¹ und R² jeweils unabhängig voneinander Wasserstoff, wobei gilt, daß R¹ und R² nicht gleichzeitig Wasserstoff sein können; eine substituierte oder unsubstituierte Alkylgruppe mit 1 bis 6 Kohlenstoffatomen oder eine substituierte oder unsubstituierte Arylgruppe mit 6 bis 10 Kohlenstoffatomen; oder R¹ und R² gemeinsam mit dem Stickstoffatom, an das sie gebunden sind, ein heterocyclisches Ringsystem;
R³ gleich R;
n gleich 0 oder 1 und
Z die Atome, die zur Vervollständigung eines 5- oder 6-gliedrigen substituierten oder unsubstituierten heterocyclischen Ringes erforderlich sind.

9. Zusammensetzung nach Anspruch 8, dadurch gekennzeichnet, daß Z für die Atome steht, die zur Vervollständigung eines Indolringes erforderlich sind.

10. Zusammensetzung nach Anspruch 8, dadurch gekennzeichnet, daß R¹ und R² jeweils Methylgruppen sind und daß R³ eine Phenylgruppe ist.
